

# United States Patent Office

3,000,943  
Patented Sept. 19, 1961

1

3,000,943

## N,N'-BIS(NITRAZAAALKYL)-N,N'-DINITRO OXAMIDES

Milton B. Frankel, Pasadena, Calif., assignor to Aerojet-General Corporation, Azusa, Calif., a corporation of Ohio  
No Drawing. Filed June 13, 1957, Ser. No. 666,270  
14 Claims. (Cl. 260—561)

This invention relates to new compositions of matter and to the preparation thereof. In particular, the invention relates to high energy N,N'-bis (nitrazaalkyl)-N,N'-dinitro oxamides having the general formula:



wherein each R is a hydrogen, alkyl, or nitroalkyl radical and each A is an alkylene radical.

The high energy oxamide compounds of this invention are particularly valuable as high explosives which can be used in any conventional explosive missile, projectile, rocket, or the like, as the main explosive charge. An example of such a missile is disclosed in United States Patent No. 2,470,162, issued May 17, 1949. One way of using the high explosives of this invention in a device such as that disclosed in United States Patent No. 2,470,162, is to pack the crystalline explosive in powder form into the warhead of the missile. Alternatively, the crystals can be first pelletized and then packed. A charge thus prepared is sufficiently insensitive to withstand the shock entailed in the ejection of a shell from a gun barrel or from a rocket launching tube under the pressure developed from ignition of a propellant charge, and can be caused to explode on operation of an impact or time fuse-mechanism firing a detonating explosive such as lead azide or mercury fulminate.

The high energy oxamide compounds of my invention are prepared by reacting N,N'-bis-(nitrazaalkyl) oxamides of the general formula:



with nitric acid, in accordance with the general reaction scheme set forth below:



wherein each R and each A is as previously defined.

To more clearly illustrate my invention, the following example is presented. It is to be understood, however, that this example is intended merely as a means of illustrating certain embodiments of my invention and that it should not be construed as limiting the scope of said invention in any way.

*Example I.—Preparation of N,N'-bis (3-nitraza-1-butyl)-N,N'-dinitro oxamide*

A mixture of 140 ml. of 100% nitric acid, 130 ml. of concentrated sulfuric acid and 9.9 g. (0.0338 mole) of N,N'-bis (3-nitraza-1-butyl) oxamide was heated at 50-55° with good stirring for 35 minutes. The reaction mixture was cooled and poured on ice. The white solid which formed was collected, washed with water, and dried to yield, as the impure product, 8.8 g. of a material having a melting point of 163-165° C., which amount corresponded to a theoretical recovery of 67.9%. The white solid was recrystallized from acetone to produce a material having a melting point of 168-169° C., as the final product. The calculated elemental analysis of the

2

product and the analysis as actually determined appear below:

Analysis.—Calcd. for  $\text{C}_8\text{H}_{14}\text{N}_8\text{O}_{10}$ : percent C, 25.13; percent H, 3.69; percent N, 29.32. Found: percent C, 25.22; percent H, 3.63; percent N, 29.11.

Reaction temperature is non-critical in the practice of this invention, the only effect of temperature variation being a corresponding increase or decrease in reaction rate.

10 The N,N'-bis (nitrazaalkyl) oxamides useful as starting materials for purposes of this invention are obtained by condensing nitraza amines, such as 3-nitraza-1-butylamine, with esters of oxalic acid, such as ethyl oxalate, as more fully disclosed in my copending U.S. patent application 15 Serial No. 666,269, filed concurrently with the present application.

The nitraza amines useful as starting materials for the preparation of the N,N'-bis (nitrazaalkyl) oxamides are generated from their corresponding strong mineral acid salts by neutralizing the strong mineral acid salts with inorganic basic salts, as for example hydroxides or carbonates of alkali or alkaline earth minerals such as sodium, calcium, etc. This method of generating nitraza amines from their strong mineral acid, i.e. hydrochloric acid, nitric acid, or the like, salts is more fully disclosed in my copending U.S. patent application Serial No. 666,273, filed concurrently with the present application.

20 The strong mineral acid salts of the nitraza amines suitable for use in the present invention are prepared by reacting corresponding nitraza isocyanates, such as 3-nitraza-1-butyl isocyanate, with aqueous strong mineral acid solutions, as more fully disclosed in my copending U.S. patent application Serial No. 666,273.

25 The above-mentioned nitraza isocyanates are prepared by reacting nitraza-acid halides, such as 4-nitrapentanoyl chloride, with alkali or alkaline earth metal azides, as for example sodium azide, or form the corresponding nitraza azides and then heating said nitraza azides under anhydrous conditions to effect rearrangement to the desired nitraza isocyanates. This method of preparing nitraza isocyanates is more fully disclosed in my copending U.S. patent application Serial No. 514,384, filed June 9, 1955.

30 The nitraza-acid halides from which the nitraza isocyanates are prepared are obtained by reacting thionyl halides, such as thionyl chloride, with appropriate nitraza-acids, as more fully disclosed in my copending U.S. patent application Serial No. 514,384. The nitraza-acids can be nitroalkyl-aza-acids which are prepared by condensing nitroalcohols with amino acids, as more fully disclosed in assignee's copending U.S. patent application Serial No. 416,385, filed March 15, 1954, or alkyl-nitraza-acids which are prepared by the acid hydrolysis of nitraza-nitriles, as disclosed in my copending U.S. patent application Serial No. 514,386, filed June 9, 1955.

35 It should be pointed out that mixtures of suitable nitraza amines can be employed in the preparation of the N,N'-bis (nitrazaalkyl) oxamides which are the starting materials in the present invention. It is thus within the purview of my invention to utilize N,N'-bis (nitrazaalkyl) oxamides of the general formula given in the reaction scheme, in which the two R's and/or the two A's are respectively different, with nitric acid, in accordance with the method of the present invention, thereby producing N,N'-bis (nitrazaalkyl)-N,N'-dinitro oxamides of the general formula claimed in which the R's and/or the A's are respectively different. For reasons of convenience and economy, however, I prefer to use N,N'-bis (nitrazaalkyl) oxamides which are symmetrical, i.e., those in which the R's and A's are respectively equivalent, as starting materials in the practice of the present invention.

40 It is preferred to carry out the nitration reaction of

this invention in the presence of a dehydrating agent, such as sulfuric acid. The dehydrating agent takes up the water of reaction thus shifting the reaction equilibrium to increase the yield. My invention is not limited to the use of sulfuric acid as the dehydrating agent. Other conventional dehydrating agents, such as acetic anhydride, phosphoric acid, or the like, can be used in the practice of my invention.

It will be appreciated that a wide variety of high energy oxamide compounds can be prepared in accordance with the method of my invention. For example, N,N'-bis (4-nitro-1-hexyl) oxamide and N,N'-bis (3-aza-3,5,5-trinitro-1-hexyl) oxamide react with nitric acid, to yield N,N'-bis (4-nitro-1-hexyl)-N,N'-dinitro oxamide and N,N'-bis (3-aza-3,5,5-trinitro-1-hexyl)-N,N'-dinitro oxamide respectively. Other members of this new series of high energy oxamide compounds are prepared simply by reacting appropriate starting materials as taught herein.

I claim:

1. As a new composition of matter, an N,N'-bis (nitroalkyl)-N,N'-dinitro oxamide having the formula:



where each R is a radical selected from the group consisting of hydrogen, lower alkyl, and lower nitroalkyl radicals and each A is a lower alkylene radical.

2. As a new composition of matter, an N,N'-bis (nitroalkyl)-N,N'-dinitro oxamide having the formula:



wherein each R is a lower alkyl radical and each A is a lower alkylene radical.

3. The composition of claim 1 in which each R is a lower nitroalkyl radical.

4. As a new composition of matter, N,N'-bis (3-nitrobutyl)-N,N'-dinitro oxamide, having the structural formula:



5. As a new composition of matter, N,N'-bis (4-nitro-1-hexyl)-N,N'-dinitro oxamide.

6. As a new composition of matter, N,N'-bis (3-aza-3,5,5-trinitro-1-hexyl)-N,N'-dinitro oxamide.

7. The method of preparing N,N'-bis (nitroalkyl)-N,N'-dinitro oxamides having the formula:



which comprises nitrating N,N'-bis (nitroalkyl) oxamides having the formula:



with nitric acid; wherein each R is a radical selected from the group consisting of hydrogen, lower alkyl, and lower nitroalkyl radicals, and each A is a lower alkylene radical.

8. The method of preparing N,N'-bis (nitroalkyl)-N,N'-dinitro oxamides having the formula:



which comprises nitrating N,N'-bis (nitroalkyl) oxamides having the formula:



with nitric acid; wherein each R is a lower alkyl radical and each A is a lower alkylene radical.

9. The method of claim 7 wherein each R is a lower nitroalkyl radical.

10. The method of preparing N,N'-bis (3-nitro-1-butyl)-N,N'-dinitro oxamide which comprises nitrating N,N'-bis (3-nitro-1-butyl) oxamide with nitric acid.

11. The method of preparing N,N'-bis (4-nitro-1-hexyl)-N,N'-dinitro oxamide which comprises nitrating N,N'-bis (4-nitro-1-hexyl) oxamide with nitric acid.

12. The method of preparing N,N'-bis (3-aza-3,5,5-trinitro-1-hexyl)-N,N'-dinitro oxamide which comprises nitrating N,N'-bis (3-aza-3,5,5-trinitro-1-hexyl) oxamide with nitric acid.

13. The method of claim 7 in which the nitration reaction is carried out in the presence of a dehydrating agent.

14. The method of claim 10 in which the nitration reaction is carried out in the presence of sulfuric acid.

No references cited.